

## UNITED STATES PATENT OFFICE

2,154,918

COUPLING COMPOUNDS FOR COLOR FORM-  
ING DEVELOPMENT

Wilhelm Schneider and Hans Loleit, Dessau, Germany, assignor to Agfa Ansco Corporation, Binghamton, N. Y., a corporation of New York

No Drawing. Application June 28, 1938, Serial No. 216,293. In Germany July 30, 1937

5 Claims. (Cl. 95—88)

The present invention relates to coupling compounds for color forming development.

Color photographic pictures have been produced with the aid of color developing dyestuff components having active methylene groups which in the development of a latent silver image by means of a developer containing a free amino-group produce a colored compound in the place of the silver image. Such dyestuff components are, for example, derivatives of aceto-acetic acid esters, of pyrazolone, of malonic acid esters, of cyanoacetophenone, of cumaranone and of hydroxythionaphthene.

It is an object of the present invention to provide an improvement in the process of producing photographic color pictures by color forming development.

A further object of the invention resides in the provision of a new and improved class of dyestuff components, color formers or coupling compounds.

Still another object of the invention is the provision of photographic developers capable of color forming development comprising compounds from the new class of color formers.

25 A further object is to provide a photographic emulsion for color forming development having incorporated compounds from the new class of color formers being fast to diffusion with respect to the silver halide emulsions.

30 Further objects of the invention will appear from the detailed specification following herein-after.

We have found that an improvement in the process of producing photographic color pictures by color forming development may be obtained by employing as the color forming compounds capable of forming a dyestuff with the oxidation product of an amino developer a pyridine derivative of the following general formula:

40



45

in which R stands for alkyl, aryl and aralkyl; X is a suitable inorganic acid radical, for example Cl, Br or I.

The pyridine nucleus may contain any suitable 50 substituents, or may be condensed with other suitable rings. These pyridine derivatives are obtained by addition of an  $\alpha$ -halogen ketone to a compound containing a tertiary nitrogen atom. Especially suitable for the purpose are pyridine, 55 and its derivatives, for example picoline, 3-amino-

pyridine or dipyridine. As ketones there may be used, for example, chloroacetophenone, bromoacetophenone, monochloracetone, symmetrical dichloracetone, bromacetophenone, para-phenylbromacetophenone, para-phenylchloracetophenone and diphenylene-para-para'-dichloromethyl ketone. The reaction of the methyl ketones and pyridine derivatives is exothermic. The operation of forming the compound may proceed in the presence or absence of a solvent. Suitable solvents are, for example, benzene or ether. By double decomposition there may be obtained from the aforesaid halogen derivatives chlorates, sulfates, or the like.

5 The new dyestuff components may be added to the developer or to the emulsion. In the development with a para-dialkylaminoaniline, yellow dyestuff pictures are produced.

When these dyestuff coupling components are mixed in the photographic layer they should be 20 made fast to diffusion in the medium of the layer by introduction of groups, which owing to their chemical structure are capable of imparting to the dyestuff components fastness to diffusion, while retaining their solubility in water. Such 25 groups are, for instance, substantive groups as described in U. S. patent application Ser. No. 72,718 filed April 4, 1936, radicals of highly polymeric carboxylic acids as described in U. S. patent application Ser. No. 90,726 filed July 15, 1936, 30 aliphatic radicals consisting of an extended saturated or unsaturated carbon chain as described in U. S. patent application Ser. No. 94,340 filed August 5, 1936, said carbon chains preferably containing radicals which impart to the finished 35 compounds solubility in water, and further other radicals of comparatively high molecular weight, which owing to their molecular dimensions prevent diffusion of the dyestuff components within the layers or from one layer to the other, such as 40 for instance polypeptide radicals (U. S. patent application Ser. No. 158,860 filed August 13, 1937), radicals of carbohydrates (U. S. patent application Ser. No. 159,518 filed August 17, 1937), radicals of natural resins (U. S. patent application 45 Ser. No. 164,499 filed September 18, 1937), sterol radicals (U. S. patent application Ser. No. 166,832 filed October 1, 1937). Furthermore there may be used compounds in which the radical of the dyestuff component itself recurs periodically (U. S. 50 patent application Ser. No. 171,701 filed October 29, 1937). Furthermore radicals may be introduced into the molecule of the dyestuff components which make the latter fast to diffusion, which radicals consist of hydroaromatic and 55

60

hydro-heterocyclic residues, then further methane radicals (U. S. patent application Ser. No. 176,058 filed November 23, 1937).

These groups may be introduced either directly 5 into the ketone, as for example into the diphenyl-acetyl chloride, into the pyridine nucleus or at any other position in the molecule, for example into the benzene nucleus of the bromacetophenone and indeed either directly or by means of 10 an amino-, hydroxyl-, or carboxyl group in the form of an acid amide or an ester.

The dyestuff components may be used in the production of both single layer materials and multi-layer materials, and in the latter case the 15 layers may be arranged on one or both sides of a support. Alternatively a mixture of emulsion particles containing different dyestuff components may be applied to the support.

In the exposed silver halide emulsion the picture 20 may be produced by simple color forming development or by reversal development as described in U. S. patent applications Ser. No. 148,731 filed June 17, 1937, and Ser. No. 100,319 filed September 11, 1936.

25 The above described coupling compounds have an improved reactivity and form the desired dyestuffs more easily than the hitherto known color formers, since the reactive methylene group appears to be activated by the vicinal pyridine 30 nucleus.

The following examples illustrate the invention:

*Example 1.*—An exposed silver halide emulsion layer is developed with a developer of the following composition:

|                                 |       |     |
|---------------------------------|-------|-----|
| (a) Para-dimethylaminoaniline   | grams | 1   |
| Anhydrous sodium carbonate      | do    | 15  |
| Sodium sulfite                  | do    | 0.1 |
| Water                           | cc    | 250 |
| 10 Potassium bromide            | grams | 1   |
| (b) Phenacylpicolinium chloride | do    | 1.8 |
| Methanol                        | cc    | 10  |

When the silver has been dissolved away a 45 yellow dyestuff picture is obtained.

*Example 2.*—An exposed silver halide emulsion layer is developed with a developer of the following composition:

|                                                                |       |     |
|----------------------------------------------------------------|-------|-----|
| (a) Para-dimethylaminoaniline                                  | grams | 1   |
| Anhydrous sodium carbonate                                     | do    | 15  |
| Sodium sulfite                                                 | do    | 0.1 |
| Water                                                          | cc    | 250 |
| Potassium bromide                                              | grams | 1   |
| (b) Phenacyl-2-hydroxy-3-nitro-5-chloro-55 pyridinium chloride | grams | 2   |
| Methanol                                                       | cc    | 10  |

A yellow dyestuff picture is obtained.

*Example 3.*—3 grams of diphenylacetylpyridinium 60 chloride of the formula



are dissolved in 25 cc. of methanol and 70 cc. of water, and the solution is added to 400 cc. of a gelatine emulsion of 5 per cent strength, and the latter is cast to form a layer. By developing the exposed layer with dimethyl-aminoaniline there 5 is obtained a yellow picture.

What we claim is:

1. In a process of producing photographic color pictures by color forming development, the improvement which comprises employing as the 10 color forming compound capable of forming a dyestuff with the oxidation product of an aromatic amino developer, a pyridine derivative of the following general formula



20 in which R is a member of the group consisting of alkyl, aryl and aralkyl, and X is an anion.

25 2. In a process of producing photographic color pictures by color forming development, the improvement which comprises employing as a color forming developer a composition of matter comprising an aqueous solution of an alkali, an aromatic amino developing agent and a pyridine derivative of the following general formula



35 in which R is a member of the group consisting of alkyl, aryl, and aralkyl, and X is an anion.

40 3. In a process of producing photographic color pictures by color forming development, the improvement which comprises employing as a light-sensitive element a photographic silver halide emulsion containing as the color forming compound capable of forming a dyestuff with the oxidation product of an aromatic amino developer, a pyridine derivative of the following 45 general formula



55 in which R is a member of the group consisting of alkyl, aryl, and aralkyl, and X is an anion, said pyridine derivative containing in its molecule a radical, which imparts thereto fastness to diffusion with respect to the binding agent of the emulsion, while retaining its solubility in aqueous liquids.

60 4. Silver halide emulsion for color photography capable of being developed in color by means of an aromatic amino developer, said silver halide emulsion containing a pyridine derivative of the following general formula



70 in which R is a member of the group consisting of alkyl, aryl, and aralkyl, and X is an anion.

75 5. A color-forming developer comprising an aqueous solution of an alkali, an aromatic amino

developing agent, and a pyridine derivative of in which R is a member of the group consisting of alkyl, aryl, and aralkyl, and X is an anion.



WILHELM SCHNEIDER.  
HANS LOEITZ.